

# UNITED STATES PATENT OFFICE.

PETER SCHMID AND KARL GROSS, OF BASEL, SWITZERLAND; SAID GROSS ASSIGNOR TO  
SAID SCHMID.

## FOAM OR FROTH DYEING-BATH FOR SILK.

1,193,430.

Specification of Letters Patent.

Patented Aug. 1, 1916.

No Drawing.

Application filed October 7, 1915. Serial No. 54,501.

*To all whom it may concern:*

Be it known that we, PETER SCHMID, a citizen of the Swiss Republic, and KARL Gross, a subject of the King of Prussia, both 5 residing in Basel, Switzerland, have invented a new and useful Foam or Froth Dyeing-Bath for Silk, of which the following is a full, clear, and exact specification.

The baths for dyeing silk hitherto employed in form of foam or froth are prepared with soapy water, whereby occurs the inconvenience that they can only be used for dyeing in a basic or neutral bath.

The present invention has for its object to 10 remove this inconvenience and is based upon the use of the liquid resulting from the boiling of silk-worm-chrysalises with water instead of soapy water for the preparation of the dyeing bath. A liquid dyeing bath prepared with this liquid can be transformed 15 into foam or froth without use of soap. The silk-worm-chrysalises necessary for the preparation of this liquid may be employed in the form of silk wastes containing silk- 20 worm-chrysalises, as for instance in form of bassinets (Italian *gallettamini*, French *pelettes*). To the water used for the preparation of the said liquid sericin can be added.

25 A dyeing bath according to this invention can be prepared as follows: 8 to 10 kg. silk-worm-chrysalises are boiled with 300 kg. water and the desired dyestuff is introduced in the liquid thus obtained. By heating 30 this bath with a steam coil, it can be trans-

formed into a froth or foam. The silk is dyed for 10 to 30 minutes in the so obtained froth or foam bath, the silk being subjected to a very little moving in the said froth or foam bath.

40 In the foregoing example the silkworm-chrysalises can be replaced by the same quantity of bassinets.

With the new dyeing bath transformed into froth or foam silk in every form can be 45 dyed as raw silk, silk wastes, silk tissues, silk spuns, etc., ungummed and not weighted or ungummed and weighted or raw and not weighted or raw and weighted.

50 What we claim is:

1. A foam or froth dyeing bath for silk prepared with the liquid obtainable by boiling of silkworm-chrysalises with water.
2. A foam or froth dyeing bath for silk prepared with the liquid obtained by boiling 55 silk wastes containing silkworm-chrysalises with water.
3. A foam or froth dyeing bath for silk prepared with the liquid obtained by boiling silkworm-chrysalises with water containing sericin.

60 In witness whereof we have hereunto signed our names this 14th day of September 1915, in the presence of two subscribing witnesses.

PETER SCHMID.  
KARL GROSS.

Witnesses:

ARNOLD ZUBER,  
ARMAND RITTER.

Copies of this patent may be obtained for five cents each, by addressing the "Commissioner of Patents,  
Washington, D. C."